



US005534045A

**United States Patent** [19]**Ogura et al.**[11] **Patent Number:** **5,534,045**[45] **Date of Patent:** **Jul. 9, 1996**[54] **WATER-ATOMIZED IRON POWDER AND METHOD**[75] Inventors: **Kuniaki Ogura; Hiroyuki Ishikawa; Yoshiaki Maeda; Kouichi Komamura, all of Chiba, Japan**[73] Assignee: **Kawasaki Steel Corporation, Japan**[21] Appl. No.: **440,913**[22] Filed: **May 15, 1995****Related U.S. Application Data**

[63] Continuation of Ser. No. 243,997, May 18, 1994, Pat. No. 5,462,577.

[30] **Foreign Application Priority Data**May 18, 1993 [JP] Japan ..... 5-115523  
Aug. 6, 1993 [JP] Japan ..... 5-196170  
Oct. 14, 1993 [JP] Japan ..... 5-256807[51] **Int. Cl.<sup>6</sup>** ..... **C22C 29/00**[52] **U.S. Cl.** ..... **75/243; 75/255**[58] **Field of Search** ..... **75/345, 255, 343, 75/243**[56] **References Cited****U.S. PATENT DOCUMENTS**4,209,320 6/1980 Kajinaga et al. ..... 75/255  
5,067,979 11/1991 Kiyota et al. ..... 75/243  
5,328,500 7/1994 Beltz et al. ..... 75/343  
5,462,577 10/1995 Ogura et al. ..... 75/345*Primary Examiner*—Scott Kastler  
*Attorney, Agent, or Firm*—Austin R. Miller[57] **ABSTRACT**

Water-atomized iron powder for powder metallurgy having a hardness of particle cross section of from about Hv 80 or higher to about 250 or lower, the iron powder having been atomized with water and dried, and having a particle surface covered with oxides which are reducible in a sintering atmosphere, and which has an oxygen content of 1.0 wt % or less.

The water-atomized iron powder can be made by an improved and simplified processing, and the cost of resulting sintered products is decreased as a result of its use.

**5 Claims, 1 Drawing Sheet**

FIG. 1



FIG. 2



## WATER-ATOMIZED IRON POWDER AND METHOD

This application is a continuation of application Ser. No. 08/243,997, filed on May 18, 1994, now U.S. Pat. No. 5,462,577.

### BACKGROUND OF THE INVENTION

#### 1. Field of the Invention

The present invention relates to an iron powder useful in water-atomized powder metallurgy, and further relates to a method of manufacturing the iron powder.

#### 2. Description of the Related Art

In general, water-atomized iron powder is made by atomizing molten steel with high pressure water. This is often followed by annealing, softening and reducing, removing oxide film from particle surfaces, and crushing. Performance of all of these steps is considered necessary. Thus, the possibility of cost reduction by eliminating processing steps is limited.

When sintered parts are made of iron powder, it is necessary to compact the iron powder with addition of lubricant and additive alloy component powders, followed by sintering the resulting green compact at a high temperature and further sizing for dimensional adjustment. Accordingly, the cost of the entire process is further increased.

Cost reduction is important. Every effort must be made to reduce manufacturing costs of, for example, automobile parts. For that purpose substantial efforts have been made.

However, omissions of any process steps, in particular, omission of annealing, softening and reducing steps has not been achieved because the water-atomized iron powder is solid due to its quenched structure and is difficult to compact. Further, although a considerable amount of oxygen is introduced into the iron powder as a sintering material, oxygen is generally considered harmful to sintered parts.

For example, although Japanese Patent Unexamined Publication No. Sho. 51-20760 discloses a method of manufacturing iron powder in which molten steel is produced in a converter and vacuum decarbonization apparatus, this method includes annealing and reducing powder atomized with water and drying.

Further, Japanese Patent Examined Publication No. Sho 56-45963 discloses a method of improving the characteristics of iron powder by mixing a finished powder that has been subjected to annealing and reducing with an atomized raw iron powder that was not subjected to annealing or reducing. Although it is desired to use atomized raw iron powder not subjected to annealing or reducing, predetermined characteristics cannot be achieved by that powder alone.

Further, although Japanese Patent Unexamined Publication No. Sho 63-157804 discloses a process for manufacturing atomized iron powder by suppressing oxidization and carburizing as much as possible by the addition of alcohol etc. to the atomizing water, the resulting iron powder contains 0.01% or more of C and is easily hardened on the cooling speed achieved by atomized water, although it contains a small amount of oxygen. The resulting iron powder cannot be compacted in dies and requires further annealing and softening.

On the other hand, it is necessary to minimize dimensional changes caused in the manufacturing process.

In particular, since the achievement of dimensional accuracy without depending upon sizing leads to the omission of process steps and accordingly to cost reduction, efforts have been made along those lines.

For example, Japanese Patent Examined Publication No. Sho 56-12304 discloses and proposes a technology for improving dimensional accuracy by particle size distribution and Japanese Patent Unexamined Publication No. Hei 3-142342 discloses and proposes technology for predicting and controlling the dimensional change in sintering according to powder configuration.

Although iron powder for powder metallurgy contains added lubricant etc. in addition to Cu powder and graphite powder, since the iron powder is moved or transported to replace the container in which it is contained, the added Cu powder and graphite powder tend to segregate, so that the components of the powder are easily dispersed. Consequently, dimensional changes caused in sintering are likely to happen, and a subsequent sizing process is conventionally indispensable.

Taking the aforesaid defects of the prior art into consideration, an important object of the invention is to provide technology for producing at low cost iron powder that is suitable for sintering. Another object of the invention is to reduce manufacturing costs of iron powder while retaining compactibility (formability). Further, another object of the invention is to lower manufacturing costs of powder as well as to manufacture an iron powder for use in powder metallurgy having stable dimensional changes in sintering, and in particular having limited dimensional dispersion with respect to the dispersion of graphite.

### SUMMARY OF THE INVENTION

The present invention relates to water-atomized iron powder for use in powder metallurgy which has a particle cross section hardness of about Hv 80 or higher to about 250 or lower when the iron powder is atomized with water and dried, further has a particle surface covered with oxides which are reducible in a sintering atmosphere, and further has an oxygen content of about 1.0 wt % or less.

In the iron powder of this invention, those particles having a particle size of from about 75  $\mu\text{m}$  or more to less than about 106  $\mu\text{m}$ , include a portion having a coefficient of particle cross-sectional configuration of about 2.5 or less and comprising in a numerical amount of about 10% or more, and the iron powder further contains particles having a particle size of about 45  $\mu\text{m}$  or less in an amount about 20 wt % or more.

In the foregoing, the coefficient of particle cross-sectional configuration of a particle is defined as a value obtained by dividing the square of the circumferential length of a particle cross section by  $4\pi$  times the cross-sectional area of the particle and is obtained by the steps mentioned below.

Step 1: Sieve iron powder and obtain particles having a diameter 75  $\mu\text{m}$ –106  $\mu\text{m}$ .

Step 2: Bury thus obtained particles into resin.

Step 3: Cut and polish thus obtained resin in an arbitrary section with iron particles and observe cross sectional configuration of iron particles using a micro-scope.

Step 4: Analyze 500–1000 particles concerning cross-sectional configuration of particles using an image analyzer and obtain a coefficient for each of said particles.

Further, water-atomized iron powder according to this invention contains elements that are more easily oxidizable than iron in an amount of 0.003 to 0.5 wt %, and has a

particle surface covered with oxides which are unreduceable in a sintering atmosphere.

This invention further relates to a method of manufacturing the iron powder covered with such oxides.

Other features of the present invention will be apparent from the accompanying detailed description and from the drawings.

#### BRIEF DESCRIPTION OF THE DRAWINGS

FIG. 1 is a chart which shows a relationship between hardness of atomized raw iron powder and the amount of C contained in the iron powder; and

FIG. 2 is another chart which shows a relationship between an amount of oxygen and the amount of Al, each in the iron powder.

#### DESCRIPTION OF THE PREFERRED EMBODIMENT

It has now been discovered that softening, annealing and reducing process steps can be eliminated under specified conditions.

Softening, annealing and reducing have been used to soften by annealing the hardened structure of the iron powder produced by atomizing with water. Raw iron powder in the water-atomized state has high hardness and is inferior in formability (compactibility) and cannot be used for powder metallurgy in that state.

The term "compactibility" refers to the green density obtained when iron powder is molded and pressed under the prevailing compacting pressure, and serves as an index for evaluating the characteristics of the green compact which is often used in powder metallurgy. When the compactibility index has a larger value, the green compact has better characteristics. Further, when iron powder is water-atomized, the iron powder particles tend to be covered with oxide films such as FeO, etc. These films interfere with formability of the iron powder and lower the strength of the sintered body. Thus, the oxide films have ordinarily been removed by softening, annealing and reducing.

The term "formability" as used herein relates to the strength of the green compact and may be represented by a "rattler value" which serves as an index for evaluating the characteristics of the green compact. A lower rattler value is preferable to a higher one.

According to this invention, water-atomized iron powder can remarkably be made with satisfactory compactibility, formability and sintering properties without the expense and burden of softening, annealing and reducing process steps.

It has been discovered that good compactibility can be achieved in atomized raw iron powder when the hardness of the particles is decreased to a Vickers hardness Hv value of about 80 to about 250.

As an example, one raw powder composed of C: 0.007 wt %, Mn: 0.005 wt %, Ni: 0.03 wt %, Cr: 0.017 wt %, Si: 0.008 wt %, P: 0.003 wt %, S: 0.002 wt % and the balance of substantial Fe had a low Vickers hardness Hv (100) of 107. When this powder was added and mixed with 1.0 wt % of zinc stearate and then compacted in metal dies at a compacting pressure of 5 t/cm<sup>2</sup>, an excellent green density of 6.81 g/cm<sup>3</sup> was obtained and both the hardness of particle cross sections and the green density had excellent values similar to those of comparable prior art iron powders which had been subjected to softening, annealing and reducing.

We have carefully examined the relationship between hardness and compactibility and have found that a green compact having advantageous green density can be obtained when the particle cross section of the iron powder had a Vickers hardness of about Hv 250. The lower the hardness of the particle cross section, the better its compactibility. It is not practical industrially to achieve a hardness less than about Hv 80 because the refining cost of the molten metal tends to be uselessly increased.

Therefore, the Vickers hardness of the particle cross section of the iron powder according to the present invention is maintained within the range of about Hv 80-250.

Such a particle cross section hardness can be obtained by reducing the amounts of harmful components such as C etc. as much as possible. As is shown in FIG. 1 of the drawings, when the amount of C is reduced the hardness of the iron powder is also reduced and approaches or betters the hardness of other finished iron powder that has been reduced and annealed.

When iron powder contains C in an amount of about 0.01 wt % or less, no significant hardening occurs even if the iron powder is atomized with water. When the content of C exceeds about 0.01 wt %, however, the powder hardness is increased. The C content is accordingly about 0.01 wt %, preferably about 0.005 wt % or less.

Mn, Ni and Cr greatly influence compactibility. As examples, various iron powders containing C in the range of about 0.01 wt % or less were atomized with water and dried, while the contents of Mn, Ni and Cr in the powders were changed through the range of about 0.40 wt % to none. When the content of Mn, Ni and Cr exceeded about 0.30 wt %, the hardness Hv (100) of the raw iron powder exceeded 250 and the iron powder was difficult to compact under pressure in metal dies. Further, sufficient green density could not be obtained. According to this invention the content of Mn, Ni and Cr should be about 0.30 wt % or less. The contents of these elements are preferably even about 0.1 wt % or less, but when they are excessively lowered, steelmaking cost is increased.

The total content of P and S should be about 0.05% or less. Although it is preferable to reduce the content of P and S as much as possible, when the total content is about 0.05% or less, no adverse hardness affect is caused.

The existence of oxygen (O) has been conventionally severely restricted; indeed O has been removed by reduction. We have discovered, however, that the presence of O is harmless to the sintering process if its content is within the parameters of this invention and if the percentage of O does not exceed a specific range. More particularly, unless the content of O exceeds about 1.0 wt %, the compactibility and formability of iron powder are satisfactory. In this case, O generally exists in combination with Fe, and when its content is within the above range, FeO is reduced to Fe in the reducing atmosphere that exists in the sintering process. Thus, the existence of O in the above range is surprisingly found to be permissible. While the O content can be any value below about 1.0 wt %, it is preferable from the viewpoint of formability to control the content of O as oxide reduced in the sintering process to about 0.5 wt % or less.

According to the present invention, Mo and/or Nb are further added in a preferable amount because these elements contribute to improvement of compactibility. Mo in a range of about 0.05 wt % to about 5.0 wt % improves compactibility and further promotes sintering and improves the strength of the sintered body. When the content of Mo exceeds about 5.0 wt %, compactibility is abruptly lowered.

Nb added in the range from about 0.005 wt % to about 0.2 wt % improves compactibility. When it is added in an amount exceeding about 0.2 wt %, however, compactibility is abruptly lowered.

Although the present invention successfully provides satisfactory iron powder for sintering, depending upon the hardness of the particles of the iron powder and a predetermined amount of oxygen contained therein, the iron powder in an atomized state has a hardness greater than that (Hv: 80-120) of generally used iron powder which has been subjected to annealing, softening and reducing. This is because of the creation of a partially hardened structure and the introduction of strain due to quenching. Therefore, it is preferable to consider and control the configuration of the iron powder particles in order to obtain good compactibility.

According to the present invention, particle configuration is represented in terms of a coefficient of particle configuration. The coefficient of particle configuration is represented by a value obtained by dividing the square of the circumference of the particle cross section by  $4\pi$  times the cross-sectional area of the particle. This value is 1 when the cross section of the particle is a perfect circle.

We have found that when particles having a coefficient of particle cross-sectional configuration of about 2.5 or less are present in an amount of about 10% or more by weight in those relatively coarse particles which have a particle size of from about 75  $\mu\text{m}$  or more to less than about 106  $\mu\text{m}$ , even if the cross section of the particles has a hardness exceeding about Hv 200, a green density of about 6.70  $\text{g}/\text{cm}^3$  or more can be obtained at a compacting pressure of 5  $\text{t}/\text{cm}^2$  when the powder is mixed with a 1 wt % of solid lubricant. This fact is highly important and advantageous.

It is important to consider those relatively coarse particles having a particle size of from about 75  $\mu\text{m}$  to about 106  $\mu\text{m}$ . The relatively coarse particles having a particle size of about 75  $\mu\text{m}$  or more greatly contribute to compactibility and have the heaviest weight when screened in normal powder metallurgy.

On the other hand, when a particle configuration is rounded, the resulting sintered body strength tends generally to be decreased. This problem can be solved by the existence in those relatively coarse particles of about 20% or more of relatively fine powder particles having a size of less than about 325 mesh, which particles are about 45  $\mu\text{m}$  or less in size.

A tensile strength of about 25  $\text{kgf}/\text{mm}^2$  or more can be obtained in a sintered body having a sintered density of 6.8  $\text{g}/\text{cm}^3$  which is obtained, for example, in such a manner that 2.0 wt % of Cu and 0.8 wt % of graphite and solid lubricant are mixed with Fe powder and compacted and then sintered at 1130° C. for 20 minutes in a  $\text{N}_2$  atmosphere. However, when particles of -325 mesh (45  $\mu\text{m}$  or less) exceed 50 wt %, compactibility is undesirably reduced.

As described above, the green density and sintered body strength of the raw powder of the present invention can be controlled in accordance with the configurations of those particles which have particle sizes of from about 75  $\mu\text{m}$  or more to less than about 106  $\mu\text{m}$ , and by considering the amount of particles having sizes of about 45  $\mu\text{m}$  or less (-325 mesh). Such particle configurations and particle size distributions can be obtained when the atomizing water has a jet pressure in a range of from about 40  $\text{kgf}/\text{cm}^2$  or higher to about 200  $\text{kgf}/\text{cm}^2$  or lower, and when the water-to-molten-metal ratio is in the range of from about 5 to 15.

The raw powder after having been atomized with water is preferably dried at about 100° to 200° C. in a non-oxidizing

atmosphere, as is usual. It is not necessary to soften, anneal or reduce the raw powder which is highly advantageous.

It is important to observe that when a sintered body is made of iron powder, its dimensional accuracy must be improved. We have found that the dimensional accuracy of sintered products can be greatly improved by the existence of specified amounts of oxides, not reduced in the sintering process, on the surfaces of the particles.

More specifically, we have discovered that the creation of FeO by oxidization in the atomizing process can be suppressed by the addition of other elements that more easily oxidizable than iron, such as Si, Al, V, Ti, Zr. These are hereinafter referred to for convenience as easy-to-oxidize elements. Iron powder having an unusual surface structure covered with oxides of the easy-to-oxidize elements can be obtained. We believe the easy-to-oxidize elements in the iron are selectively oxidized so that oxide films are formed on the surface of the iron powder and serve as protective films.

Although the reason why dimensional accuracy can be improved by the existence of the oxides of the easy-to-oxidize elements on the surface of iron powder is not yet clarified, we believe that the diffusion of carbon from graphite added in the sintering process into the particles of the iron powder is suppressed. Thus, the amount of C invading and diffusing into the iron powder is kept substantially at a specific level regardless of changes of the amount of added graphite or changes of its particle size. As a result, the amount of so-called expansion due to Cu is also stabilized.

With this arrangement, the dispersion of dimensional changes of a Fe-Cu-C system which is sensitive to the dispersion of graphite can be suppressed to a low level.

The amount of oxygen in the form of FeO on the powder is simultaneously reduced by the addition of the easy-to-oxidize elements, whereby the formability of the iron powder is further improved.

FIG. 2 of the drawings shows a typical relationship between the amount of Al dissolved in the molten steel and the content of O in a water-atomized raw iron powder.

The easy-to-oxidize elements in accordance with this invention include Si, Al, V, Ti and Zr. They may be present or added independently or as a mixture. Preferable ranges of addition are as follows: Si: about 0.01-about 0.1 wt %, Al: about 0.003-about 0.05 wt %,

V: about 0.008-about 0.5 wt %, Ti: about 0.003-about 0.1 wt %,

Zr: about 0.008-about 0.1 wt %.

The content of the easy-to-oxidize elements is better to be from about 0.003 wt % or more to about 0.5 wt %. When this amount is less than about 0.003 wt %, there is substantially no reduction of oxygen content, whereas an amount exceeding about 0.5 wt % tends to increase the content of oxygen, and resulting sintered body strength is abruptly decreased.

It is important to observe that to achieve improvement of dimensional accuracy of the product, the easy-to-oxidize elements must have an oxidizing ratio of about 20 wt % or more. When the oxidizing ratio is less than about 20 wt % there is less reduction of the variable range of dimensional changes in sintering with respect to the dispersion of added graphite. Even in this case, however, the oxygen content in the iron powder is limited to about 1% and preferably to about 0.5% or less, for the purpose of maintaining formability.

In order for the easy-to-oxidize element (Si, Al, V, Ti, Zr) to be added to molten steel to thereby create suitable oxide

films on the surface of iron powder, the iron powder is atomized with water in a non-oxidizing gas atmosphere containing oxygen ( $O_2$ ) with a concentration of about 5.0 vol % or less and dried in hydrogen, nitrogen or vacuum.

## EXAMPLES

### Example 1

Molten metal containing C: 0.002 wt %, Mn: 0.002 wt %, Ni: 0.006 wt %, Cr: 0.013 wt %, Si: 0.005 wt %, P: 0.002 wt %, S: 0.002 wt % was prepared in such a manner that molten steel was refined in a converter and decarbonized by the use of a vacuum decarbonizing apparatus. This molten metal was atomized with water at a water pressure of 75 kgf/cm<sup>2</sup> and a water-to-molten-steel ratio of 10. The resulting powder was dried at 125° C. in an atmosphere of  $N_2$  and then screened to 1000  $\mu$ m or less without being annealed and reduced.

The hardness of the powder was determined by measuring the cross section of the powder in terms of Vickers hardness with a load of 100 g. The coefficient of cross-sectional configuration of the particles was measured by means of an image processing apparatus. Green density was measured in such a manner that 1.0 wt % of zinc stearate was added to and mixed with raw powder and a tablet having a diameter of 11.3 mm $\phi$  was compacted at a pressure of 5 t/cm<sup>2</sup>. Sintered body strength was determined by measuring tensile strength of Fe-2.0 Cu-0.8 composition with a sintered density of 6.80 Mg/m<sup>3</sup> which was obtained in such a manner that a mixed powder of raw iron powder, Cu powder, graphite powder and solid lubricant was compacted and then sintered at 1130° C. in an endothermic gas (propane converted gas) atmosphere for 20 minutes.

Comparative Example 1 was obtained by subjecting commercially available water-atomized iron powder for sintering which had been reduced and annealed to the same process as the aforesaid. Table 1-1 shows chemical composition of the iron powders and Table 1-2 shows powder hardness, sintered body strength and the like.

Example 1 can obtain the powder hardness, green density and sintered body characteristics which are substantially the same as those of the conventional iron powder of Comparative Example 1 even without annealing or reducing.

TABLE 1-1

|                       | Chemical composition of raw powder (wt %) |       |       |       |       |       |       |
|-----------------------|-------------------------------------------|-------|-------|-------|-------|-------|-------|
|                       | C                                         | Mn    | Ni    | Cr    | Si    | P     | S     |
| Example 1             | 0.002                                     | 0.002 | 0.006 | 0.013 | 0.005 | 0.002 | 0.002 |
| Comparative example 1 | 0.001                                     | 0.11  | 0.013 | 0.008 | 0.01  | 0.014 | 0.008 |

### Examples 2-11, Comparative Examples 2-9

After having been refined in a converter or an electric furnace, molten metal containing C: 0.002-0.04 wt %, Mn: 0.4 wt % or less, Ni: 0.4 wt % or less, Cr: 0.4 wt % or less, Si: 0.005-0.03 wt %, P: 0.002-0.025 wt %, S: 0.002-0.03 wt % was prepared by use of a vacuum degassing apparatus. The molten metal was atomized with water under a water pressure of 30-250 kgf/cm<sup>2</sup> and with a water to molten steel ratio of 10. The thus obtained powder was dried at 125° C. in an  $N_2$  atmosphere, except in Comparative Example 7. Comparative Example 7 was dried at 125° C. in the atmosphere. These raw powders were screened to 1000  $\mu$ m or less without being annealed or reduced.

Particle hardness, coefficient of particle cross-sectional configurations of the raw powders, green density and sintered body strength were measured using the same methods as Example 1.

Table 2-1 shows chemical composition of raw iron powders of Examples 2-11 and Comparative Examples 2-9. Table 2-2 shows powder hardness, atomized water pressure, ratio of particles having a coefficient of configuration of 2.5 or less in the particles having a particle size of 75-106  $\mu$ m, ratio of particles having a size of -325# (45  $\mu$ m or less), green density not subjected to a finishing reduction, and sintered body strength.

Although any of Examples 2-11 exhibits a practically applicable green density and sintered body strength, Comparative Examples 2-7 have the composition of raw powders which exceeds a proper range. Thus, the hardness of particles is Hv (100) 250 or higher and a green density of 6.70 Mg/m<sup>3</sup> or more cannot be obtained at a compacting pressure of 5 t/cm<sup>2</sup>. Since Comparative Example 8 has an atomizing pressure exceeding a proper range, the ratio of the particles having a coefficient of configuration of 2.5 or less is 10% or less in the particles having a particle size of 75-106  $\mu$ m. Thus, a green density of 6.70 Mg/m<sup>3</sup> or more cannot be obtained at a compacting pressure of 5 t/cm<sup>2</sup>. Since Comparative Example 9 has an atomizing pressure exceeding a proper range, particles of -325# are 20% or less and thus a sintered body strength of 300 MPa cannot be obtained at a sintered body density of 6.80 Mg/m<sup>3</sup>.

TABLE 2-1

|           | Chemical composition of raw powder (wt %) |       |       |       |       |       |       |      |
|-----------|-------------------------------------------|-------|-------|-------|-------|-------|-------|------|
|           | C                                         | Mn    | Ni    | Cr    | Si    | P     | S     | O    |
| Example 2 | 0.002                                     | 0.001 | 0.005 | 0.001 | 0.005 | 0.001 | 0.002 | 0.61 |
| Example 3 | 0.006                                     | 0.005 | 0.011 | 0.01  | 0.010 | 0.005 | 0.002 | 0.45 |
| Example 4 | 0.010                                     | 0.01  | 0.011 | 0.02  | 0.018 | 0.006 | 0.009 | 0.47 |
| Example 5 | 0.010                                     | 0.012 | 0.013 | 0.025 | 0.020 | 0.006 | 0.008 | 0.45 |
| Example 6 | 0.006                                     | 0.29  | 0.005 | 0.001 | 0.005 | 0.002 | 0.002 | 0.65 |
| Example 7 | 0.006                                     | 0.05  | 0.29  | 0.002 | 0.007 | 0.001 | 0.003 | 0.52 |

TABLE 1-2

| Powder hardness (Hv(100)) | Pressure of atomizing water (kgf/cm <sup>2</sup> ) | Number % of Particles having coefficient of configuration of 2.5 or less (Particles size 75-106 $\mu$ m) | wt % of Particle through 325 mesh (-45 $\mu$ m) | Green density compacted at 5t/cm <sup>2</sup> (Mg/m <sup>3</sup> ) | Sintered body strength Sintered body density 6.8 Mg/m <sup>3</sup> (MPa) |
|---------------------------|----------------------------------------------------|----------------------------------------------------------------------------------------------------------|-------------------------------------------------|--------------------------------------------------------------------|--------------------------------------------------------------------------|
| Example 1                 | 102                                                | 75                                                                                                       | 35                                              | 27                                                                 | 6.93                                                                     |
| Comparative example 1     | 100                                                | —                                                                                                        | —                                               | 21                                                                 | 6.94                                                                     |

TABLE 2-1-continued

|                       | Chemical composition of raw powder (wt %) |       |       |       |       |       |       |      |
|-----------------------|-------------------------------------------|-------|-------|-------|-------|-------|-------|------|
|                       | C                                         | Mn    | Ni    | Cr    | Si    | P     | S     | O    |
| Example 8             | 0.007                                     | 0.006 | 0.004 | 0.3   | 0.006 | 0.004 | 0.002 | 0.62 |
| Example 9             | 0.005                                     | 0.004 | 0.004 | 0.003 | 0.005 | 0.015 | 0.019 | 0.51 |
| Example 10            | 0.004                                     | 0.004 | 0.005 | 0.004 | 0.005 | 0.002 | 0.002 | 0.55 |
| Example 11            | 0.004                                     | 0.003 | 0.005 | 0.003 | 0.005 | 0.003 | 0.003 | 0.55 |
| Example 12            | 0.005                                     | 0.004 | 0.003 | 0.002 | 0.006 | 0.004 | 0.004 | 0.55 |
| Comparative Example 2 | 0.032                                     | 0.01  | 0.013 | 0.2   | 0.029 | 0.007 | 0.011 | 0.41 |
| Comparative Example 3 | 0.005                                     | 0.38  | 0.003 | 0.004 | 0.005 | 0.002 | 0.002 | 0.7  |
| Comparative Example 4 | 0.004                                     | 0.004 | 0.41  | 0.003 | 0.005 | 0.002 | 0.003 | 0.53 |
| Comparative Example 5 | 0.004                                     | 0.003 | 0.003 | 0.42  | 0.005 | 0.002 | 0.002 | 0.68 |
| Comparative Example 6 | 0.003                                     | 0.003 | 0.004 | 0.004 | 0.008 | 0.025 | 0.030 | 0.51 |
| Comparative Example 7 | 0.003                                     | 0.002 | 0.002 | 0.003 | 0.003 | 0.002 | 0.004 | 1.2  |
| Comparative Example 8 | 0.003                                     | 0.003 | 0.004 | 0.004 | 0.008 | 0.005 | 0.005 | 0.65 |
| Comparative Example 9 | 0.003                                     | 0.003 | 0.004 | 0.004 | 0.008 | 0.005 | 0.005 | 0.6  |

19 was dried at 125° C. in the atmosphere. These raw powders were screened to 1000 µm or less without being annealed or reduced.

Particle hardness, coefficient of particle cross-sectional configuration of the raw powders, green density and sintered body strength were measured by the same methods as Example 1. Table 3-1 shows chemical composition of the raw iron powders of Examples 12-24 and Comparative Examples 10-19, and Table 3-2 shows powder hardness, atomized water pressure, ratio of the particles having a coefficient of configuration of 2.5 or less in the particles having a particle size of 75-106 µm, ratio of particles having a size of -325# (45 µm or less), green density, and sintered body strength of these examples and comparative examples.

5 10 15 Although Examples 12-24 exhibit a practically applicable green density and sintered body strength, Comparative Examples 10-16 have compositions of raw powders which exceed a proper range. Thus, the hardness of the particles is 250 or more and the green density of 6.70 Mg/m<sup>3</sup> or more cannot be obtained at a compacting pressure of 5 t/cm<sup>2</sup>. Since Comparative Example 17 has an atomizing pressure exceeding a proper range, the ratio of the particles having a coefficient of configuration of 2.5 or less is 10% or less in the particles having a particle size of 75-106 µm. Thus, a green

20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365

TABLE 3-1

|                        | Chemical composition of raw powder (wt %) |      |       |       |       |       |       |     |       |      |
|------------------------|-------------------------------------------|------|-------|-------|-------|-------|-------|-----|-------|------|
|                        | C                                         | Mn   | Ni    | Cr    | Si    | P     | S     | Mo  | Nb    | O    |
| Example 12             | 0.003                                     | 0.03 | 0.005 | 0.01  | 0.006 | 0.008 | 0.006 | 0.5 | 0.005 | 0.51 |
| Example 13             | 0.004                                     | 0.04 | 0.01  | 0.001 | 0.006 | 0.01  | 0.005 | 1.0 | 0.007 | 0.45 |
| Example 14             | 0.005                                     | 0.03 | 0.01  | 0.011 | 0.007 | 0.008 | 0.006 | 2.0 | 0.006 | 0.52 |
| Example 15             | 0.003                                     | 0.05 | 0.008 | 0.012 | 0.008 | 0.008 | 0.006 | 4.0 | 0.006 | 0.44 |
| Example 16             | 0.002                                     | 0.05 | 0.007 | 0.004 | 0.01  | 0.009 | 0.008 | 0.5 | 0.01  | 0.5  |
| Example 17             | 0.002                                     | 0.04 | 0.011 | 0.006 | 0.006 | 0.008 | 0.006 | 0.5 | 0.05  | 0.42 |
| Example 18             | 0.002                                     | 0.04 | 0.008 | 0.008 | 0.006 | 0.008 | 0.006 | 0.5 | 0.05  | 0.42 |
| Example 19             | 0.002                                     | 0.04 | 0.011 | 0.006 | 0.006 | 0.008 | 0.006 | 0.2 | 0.15  | 0.42 |
| Example 20             | 0.006                                     | 0.01 | 0.005 | 0.005 | 0.02  | 0.01  | 0.015 | 0.3 | 0.02  | 0.35 |
| Example 21             | 0.01                                      | 0.02 | 0.005 | 0.005 | 0.008 | 0.007 | 0.002 | 0.2 | 0.02  | 0.5  |
| Example 22             | 0.003                                     | 0.25 | 0.006 | 0.005 | 0.008 | 0.008 | 0.006 | 0.1 | 0.03  | 0.5  |
| Example 23             | 0.002                                     | 0.03 | 0.25  | 0.005 | 0.008 | 0.007 | 0.006 | 0.2 | 0.008 | 0.47 |
| Example 24             | 0.002                                     | 0.03 | 0.012 | 0.25  | 0.008 | 0.007 | 0.006 | 0.5 | 0.009 | 0.53 |
| Comparative Example 10 | 0.03                                      | 0.04 | 0.011 | 0.006 | 0.006 | 0.008 | 0.006 | 0.2 | 0.15  | 0.42 |
| Comparative Example 11 | 0.002                                     | 0.4  | 0.008 | 0.01  | 0.01  | 0.01  | 0.009 | 0.2 | 0.007 | 0.5  |
| Comparative Example 12 | 0.005                                     | 0.1  | 0.4   | 0.01  | 0.01  | 0.008 | 0.009 | 0.5 | 0.007 | 0.56 |
| Comparative Example 13 | 0.004                                     | 0.06 | 0.01  | 0.4   | 0.01  | 0.008 | 0.009 | 0.5 | 0.007 | 0.55 |
| Comparative Example 14 | 0.003                                     | 0.11 | 0.01  | 0.009 | 0.01  | 0.025 | 0.03  | 0.5 | 0.008 | 0.61 |
| Comparative Example 15 | 0.003                                     | 0.1  | 0.01  | 0.011 | 0.008 | 0.007 | 0.008 | 6.0 | 0.01  | 0.57 |
| Comparative Example 16 | 0.003                                     | 0.1  | 0.01  | 0.01  | 0.007 | 0.011 | 0.007 | 0.4 | 0.3   | 0.59 |
| Comparative Example 17 | 0.005                                     | 0.02 | 0.005 | 0.005 | 0.008 | 0.007 | 0.002 | 0.2 | 0.02  | 0.5  |
| Comparative Example 18 | 0.005                                     | 0.02 | 0.005 | 0.005 | 0.008 | 0.007 | 0.002 | 0.2 | 0.02  | 0.5  |
| Comparative Example 19 | 0.002                                     | 0.11 | 0.011 | 0.009 | 0.01  | 0.011 | 0.008 | 0.1 | 0.008 | 1.5  |

TABLE 3-2

|                    | Powder hardness (Hv(100)) | Pressure of atomizing water (kgf/cm <sup>2</sup> ) | Number % of Particles having coefficient of configuration of 2.5 or less (Particles size 75~106 $\mu$ m) | wt % of Particle through 325 mesh (-45 $\mu$ m) | Green density at 5t/cm <sup>2</sup> (Mg/m <sup>3</sup> ) | Sintered body strength Sintered body density 6.8 Mg/m <sup>3</sup> (MPa) |
|--------------------|---------------------------|----------------------------------------------------|----------------------------------------------------------------------------------------------------------|-------------------------------------------------|----------------------------------------------------------|--------------------------------------------------------------------------|
| Example 12         | 121                       | 120                                                | 35                                                                                                       | 27                                              | 6.87                                                     | 550                                                                      |
| Example 13         | 125                       | 120                                                | 33                                                                                                       | 30                                              | 6.9                                                      | 610                                                                      |
| Example 14         | 127                       | 120                                                | 35                                                                                                       | 32                                              | 6.91                                                     | 750                                                                      |
| Example 15         | 130                       | 120                                                | 37                                                                                                       | 32                                              | 6.92                                                     | 820                                                                      |
| Example 16         | 128                       | 120                                                | 30                                                                                                       | 31                                              | 6.89                                                     | 555                                                                      |
| Example 17         | 125                       | 120                                                | 30                                                                                                       | 30                                              | 6.88                                                     | 550                                                                      |
| Example 18         | 170                       | 150                                                | 28                                                                                                       | 33                                              | 6.85                                                     | 590                                                                      |
| Example 19         | 175                       | 150                                                | 29                                                                                                       | 35                                              | 6.88                                                     | 510                                                                      |
| Example 20         | 180                       | 150                                                | 28                                                                                                       | 32                                              | 6.8                                                      | 530                                                                      |
| Example 21         | 220                       | 100                                                | 30                                                                                                       | 36                                              | 6.75                                                     | 515                                                                      |
| Example 22         | 177                       | 100                                                | 25                                                                                                       | 35                                              | 6.78                                                     | 480                                                                      |
| Example 23         | 180                       | 200                                                | 10                                                                                                       | 45                                              | 6.77                                                     | 500                                                                      |
| Example 24         | 164                       | 40                                                 | 72                                                                                                       | 20                                              | 6.8                                                      | 540                                                                      |
| Comparative ex. 10 | 310                       | 120                                                | 30                                                                                                       | 30                                              | 6.5                                                      | 505                                                                      |
| Comparative ex. 11 | 280                       | 120                                                | 32                                                                                                       | 31                                              | 6.55                                                     | 500                                                                      |
| Comparative ex. 12 | 270                       | 120                                                | 31                                                                                                       | 31                                              | 6.53                                                     | 540                                                                      |
| Comparative ex. 13 | 285                       | 120                                                | 29                                                                                                       | 32                                              | 6.61                                                     | 545                                                                      |
| Comparative ex. 14 | 288                       | 120                                                | 28                                                                                                       | 30                                              | 6.6                                                      | 550                                                                      |
| Comparative ex. 15 | 268                       | 120                                                | 30                                                                                                       | 28                                              | 6.52                                                     | 830                                                                      |
| Comparative ex. 16 | 280                       | 120                                                | 29                                                                                                       | 25                                              | 6.51                                                     | 530                                                                      |
| Comparative ex. 17 | 125                       | 250                                                | 5                                                                                                        | 55                                              | 6.65                                                     | 510                                                                      |
| Comparative ex. 18 | 130                       | 30                                                 | 80                                                                                                       | 10                                              | 6.89                                                     | 250                                                                      |
| Comparative ex. 19 | 135                       | 120                                                | 29                                                                                                       | 21                                              | 6.92                                                     | 280                                                                      |

## Examples 25-29, Comparative Examples 20-22

After having been refined in a converter or an electric furnace, molten metal containing C: 0.01 wt % or less, Mn: 0.1 wt % or less, Ni: 0.1 wt % or less, Cr: 0.1 wt % or less, Si: 0.02 wt % or less, P: 0.02 wt % or less, S: 0.02 wt % or less, Al: 0.1 wt % or less was prepared by use of a vacuum degassing apparatus. This molten metal was atomized with water under water pressure of 120 kgf/cm<sup>2</sup> and a water-to-molten-steel ratio of 10. The thus obtained raw powders were dried at 125°C. in an N<sub>2</sub> atmosphere. The raw powders were screened to 250  $\mu$ m or less without being annealed or reduced. Table 4 shows particle hardness, chemical compo-

55 sition of iron powders, green density, rattler value, tensile strength, and impact value. Examples 25-29 have an oxygen content of 0.4% or less because it contains a proper amount of Al. As a result, these examples exhibit a green density of 6.7 g/m<sup>3</sup> or more, sintered body strength of 40 kgf/mm<sup>2</sup> or more and rattler value of 1.5% or less, but Comparative Examples 20, 22 exhibit a rattler value of 1.5% or more and a lowered formability because they contain Al in an amount exceeding a proper range although having a green density of 6.7 g/m<sup>3</sup> or more. Further, Comparative Example 21 has a green density of 6.5 g/m<sup>3</sup> or less because it has a hardness exceeding Hv 250.

TABLE 4

|             | Chemical composition of iron powder (wt %) |       |       | Fe and other indispensable impurities | Hardness Hv (100 g) | Green                        | Rattler   | Impact value (kg-m/cm <sup>2</sup> ) |      |
|-------------|--------------------------------------------|-------|-------|---------------------------------------|---------------------|------------------------------|-----------|--------------------------------------|------|
|             | Al (%)                                     | C (%) | O (%) |                                       |                     | density (g/cm <sup>3</sup> ) | value (%) |                                      |      |
| Example 25  | 0.006                                      | 0.003 | 0.38  | the remainder                         | 120                 | 6.70                         | 0.85      | 42                                   | 0.9  |
| Example 26  | 0.010                                      | 0.004 | 0.36  | the remainder                         | 124                 | 6.75                         | 0.9       | 43                                   | 0.95 |
| Example 27  | 0.021                                      | 0.003 | 0.35  | the remainder                         | 130                 | 6.74                         | 1.0       | 44                                   | 0.88 |
| Example 28  | 0.031                                      | 0.002 | 0.33  | the remainder                         | 133                 | 6.80                         | 1.2       | 43                                   | 0.87 |
| Example 29  | 0.046                                      | 0.002 | 0.30  | the remainder                         | 135                 | 6.81                         | 1.4       | 41                                   | 0.85 |
| Comparative | 0.001                                      | 0.003 | 0.55  | the remainder                         | 135                 | 6.71                         | 1.9       | 40                                   | 0.83 |
| Example 20  |                                            |       |       |                                       |                     |                              |           |                                      |      |
| Comparative | 0.020                                      | 0.025 | 0.34  | the remainder                         | 270                 | 6.45                         | 3.8       | 32                                   | 0.65 |
| Example 21  |                                            |       |       |                                       |                     |                              |           |                                      |      |
| Comparative | 0.070                                      | 0.002 | 0.30  | the remainder                         | 140                 | 6.80                         | 1.5       | 31                                   | 0.63 |
| Example 22  |                                            |       |       |                                       |                     |                              |           |                                      |      |

Examples 30-36, Comparative Examples 23-26

After having been refined in a converter or an electric furnace, molten metal containing C: 0.01 wt % or less, Mn: 0.1 wt % or less, Ni: 0.1 wt % or less, Cr: 0.1 wt % or less, Si: 0.02 wt % or less, P: 0.02 wt % or less, S: 0.02 wt % or less, Si+Ti+Zr: 0.2 wt % or less was prepared by use of a vacuum degassing apparatus. This molten metal was atomized at a water pressure of 130 kgf/cm<sup>2</sup>. The thus obtained raw powders were dried at 125° C. in an N<sub>2</sub> atmosphere. The raw powders were screened to 250 µm or less without being annealed or reduced.

Table 5 shows particle hardness, chemical composition of iron powders, green density, rattler value, tensile strength and impact value.

Examples 30-36 have an oxygen content of 0.5% or less because they contain a proper amount of any of Si, Ti or Zr. As a result, these Examples exhibit a sintered body strength of 40 kgf/mm<sup>2</sup> or more and rattler value of 1.5% or less, but Comparative Examples 23 exhibits a rattler value of 1.5% or more and a lowered formability because it contains Si, Ti, Zr in an amount less than the proper range. Comparative Example 24 has a green density of 6.5 g/m<sup>3</sup> or less because it has a particle hardness exceeding Hv 250. Further, Comparative Examples 25 and 26, which contain Si, Ti, Zr in an amount exceeding a proper range, have a lowered sintered body strength.

30

35

40

TABLE 5-1

|                    | Composition value of molten steel (wt %) |        |        |       |       | Atomizing conditions  |                              | Analyzed value of atomized raw powder (wt %) |        |        |       |       |
|--------------------|------------------------------------------|--------|--------|-------|-------|-----------------------|------------------------------|----------------------------------------------|--------|--------|-------|-------|
|                    |                                          |        |        |       |       | Water to molten steel | Atmosphere (O <sub>2</sub> ) |                                              |        |        |       |       |
|                    | Si (%)                                   | Ti (%) | Zr (%) | C (%) | O (%) |                       |                              | Si (%)                                       | Ti (%) | Zr (%) | C (%) | O (%) |
| Example 30         | 0.020                                    | 0.002  | 0.002  | 0.008 | 0.010 | 8                     | N <sub>2</sub> (1.0)         | 0.020                                        | 0.002  | 0.002  | 0.002 | 0.38  |
| Example 31         | 0.013                                    | 0.002  | 0.002  | 0.009 | 0.007 | 7.5                   | N <sub>2</sub> (1.0)         | 0.012                                        | 0.002  | 0.002  | 0.003 | 0.45  |
| Example 32         | 0.032                                    | 0.002  | 0.003  | 0.010 | 0.005 | 7                     | N <sub>2</sub> (0.5)         | 0.030                                        | 0.002  | 0.003  | 0.004 | 0.33  |
| Example 33         | 0.004                                    | 0.020  | 0.022  | 0.008 | 0.009 | 7                     | N <sub>2</sub> (1.0)         | 0.004                                        | 0.020  | 0.020  | 0.002 | 0.35  |
| Example 34         | 0.004                                    | 0.016  | 0.015  | 0.007 | 0.006 | 7.5                   | N <sub>2</sub> (0.5)         | 0.004                                        | 0.015  | 0.015  | 0.002 | 0.40  |
| Example 35         | 0.001                                    | 0.002  | 0.018  | 0.005 | 0.007 | 7                     | Ar(0.3)                      | 0.001                                        | 0.002  | 0.017  | 0.003 | 0.45  |
| Example 36         | 0.021                                    | 0.021  | 0.015  | 0.006 | 0.005 | 6.5                   | N <sub>2</sub> (2.0)         | 0.020                                        | 0.020  | 0.015  | 0.003 | 0.40  |
| Comparative ex. 23 | 0.003                                    | <0.001 | <0.001 | 0.005 | 0.020 | 7                     | N <sub>2</sub> (2.0)         | 0.002                                        | <0.001 | <0.001 | 0.003 | 0.60  |
| Comparative ex. 24 | 0.015                                    | 0.010  | 0.002  | 0.035 | 0.007 | 7                     | N <sub>2</sub> (1.0)         | 0.015                                        | 0.010  | 0.002  | 0.020 | 0.40  |
| Comparative ex. 25 | 0.121                                    | 0.010  | 0.005  | 0.007 | 0.007 | 8                     | N <sub>2</sub> (1.0)         | 0.120                                        | 0.010  | 0.005  | 0.003 | 0.35  |
| Comparative ex. 26 | 0.055                                    | 0.150  | 0.033  | 0.007 | 0.005 | 7.5                   | N <sub>2</sub> (1.0)         | 0.050                                        | 0.030  | 0.030  | 0.002 | 0.38  |

TABLE 5-2

|                        | Characteristic of green compact |                                    | Characteristic of sintered body |                                        |                                      |
|------------------------|---------------------------------|------------------------------------|---------------------------------|----------------------------------------|--------------------------------------|
|                        | Hardness HV (100 g)             | Green density (g/cm <sup>3</sup> ) | Rattler value (%)               | Tensile strength (kg/mm <sup>2</sup> ) | Impact value (kg·m/cm <sup>2</sup> ) |
| Example 30             | 130                             | 6.72                               | 0.8                             | 44                                     | 0.95                                 |
| Example 31             | 125                             | 6.75                               | 0.9                             | 42                                     | 0.92                                 |
| Example 32             | 130                             | 6.76                               | 1.0                             | 45                                     | 0.88                                 |
| Example 33             | 130                             | 6.82                               | 1.1                             | 43                                     | 0.87                                 |
| Example 34             | 128                             | 6.80                               | 1.3                             | 41                                     | 0.85                                 |
| Example 35             | 135                             | 6.71                               | 1.2                             | 40                                     | 0.8                                  |
| Example 36             | 138                             | 6.60                               | 0.9                             | 42                                     | 0.85                                 |
| Comparative Example 23 | 135                             | 6.70                               | 2.0                             | 39                                     | 0.75                                 |
| Comparative Example 24 | 270                             | 6.45                               | 3.8                             | 31                                     | 0.6                                  |
| Comparative Example 25 | 150                             | 6.60                               | 1.4                             | 29                                     | 0.5                                  |
| Comparative Example 26 | 145                             | 6.63                               | 1.4                             | 30                                     | 0.55                                 |

## Examples 37, Comparative Example 27

Molten metal containing C: 0.004 wt %, Mn: 0.03 wt %, Ni: 0.005 wt %, Cr: 0.01 wt %, Si: 0.006 wt %, P: 0.008 wt %, S: 0.006 wt %, Al: 0.004 wt % was prepared in such a manner that molten steel was refined in a converter and decarbonized by use of a vacuum decarbonizing apparatus. This molten metal was atomized with jet water having a water pressure of 70 kgf/cm<sup>2</sup> in an N<sub>2</sub> atmosphere having an oxygen concentration of 0.5%. The thus obtained powder was dried at 180° C. in a H<sub>2</sub> atmosphere and then screened to 250 µm or less without being annealed and reduced.

Green density was measured in such a manner that 1.0 wt % of zinc stearate was added to and mixed with raw powder and a tablet having a diameter of 11.3 mmφ was compacted at a pressure of 5 t/cm<sup>2</sup>. Sintered body strength was measured in such a manner that powder prepared by mixing raw iron powder, Cu powder, graphite powder and zinc stearate as lubricant was compacted to a JSMP standard tensile strength test piece and the tensile strength of a sintered body

20 outside diameter of 60φ, inside diameter of 25φ, height of 10 mm, and green density of 6.85 g/cm<sup>3</sup> and sintered at 1130° C. in an endothermic gas (propane converted gas) atmosphere for 20 minutes.

Comparative Example 27 was obtained by subjecting 25 commercially available water-atomized iron powder for powder metallurgy which had been reduced and annealed to the same process as the aforesaid one. Table 6-1 shows a chemical composition of iron powders and a ratio of oxidation of easy-to-oxidize elements, and Table 6-2 shows a hardness of particle cross section, green density, sintered body strength and variable range of dimensional changes. Example 37 not only has substantially the same green 30 density as that of Comparative Example 27 but also exhibits a variable range of dimensional changes superior to that of the iron powder of Comparative Example 27 regardless of that Example 37 is not annealed and reduced.

TABLE 6-1

|                        | Chemical composition of raw powder (wt %) |      |       |       |       |       |       |       | Ratio of oxidization of easy-to-oxidize elements (%) |
|------------------------|-------------------------------------------|------|-------|-------|-------|-------|-------|-------|------------------------------------------------------|
|                        | C                                         | Mn   | Ni    | Cr    | Si    | P     | S     | Al    |                                                      |
| Example 37             | 0.004                                     | 0.03 | 0.005 | 0.01  | 0.006 | 0.008 | 0.006 | 0.004 | 0.45                                                 |
| Comparative Example 27 | 0.001                                     | 0.11 | 0.011 | 0.009 | 0.01  | 0.012 | 0.009 | —     | 35                                                   |

TABLE 6-2

|                        | Green density compacted at 60           | Sintered body strength Sintered body density 65 | Variable range of dimensional changes (%) | Hardness (%) |
|------------------------|-----------------------------------------|-------------------------------------------------|-------------------------------------------|--------------|
|                        | Si/cm <sup>2</sup> (Mg/m <sup>3</sup> ) | 6.8 Mg/m <sup>3</sup> (MPa)                     |                                           |              |
| Example 37             | 6.86                                    | 440                                             | 0.06                                      | 110          |
| Comparative Example 27 | 6.91                                    | 430                                             | 0.2                                       | 100          |

(sintered density: 6.8 Mg/m<sup>3</sup>, a composition of Fe-2.0 Cu-0.8 C) obtained by sintering the test piece at 1130° in an endothermic gas (propane converted gas) atmosphere for 20 minutes was measured. A dimensional change in sintering was examined with respect to amounts of graphite of two levels or Fe-2.0% Cu-0.8% Gr and Fe-2.0% Cu-1.0% Gr and a difference of the respective changes of sintered dimension was used as a "variable range of dimensional changes". At that time, the test piece was formed to a ring shape with an

## Examples 38-52, Comparative Examples 28-31

60 After having been refined in a converter or an electric furnace, molten metal containing C: 0.01 wt % or less, Mn: 0.1 wt % or less, Ni: 0.1 wt % or less, Cr: 0.1 wt % or less, P: 0.02 wt % or less, S: 0.02 wt % or less, a total amount of Si, Al, Ti and V: 0.6 wt % or less was prepared by use of a vacuum degassing apparatus. This molten metal was atomized with water having a pressure of 100 kgf/cm<sup>2</sup> in an N<sub>2</sub> atmosphere with an oxygen concentration of 10% or less.

The thus obtained raw powders were dried at 100°–300° C. in H<sub>2</sub>, N<sub>2</sub> or vacuum for 60 minutes and then screened to 250 µm or less without being annealed and reduced.

Green density, sintered body strength and variable range of dimensional changes of sintered body were measured by the same methods as those of Example 37. Table 7 shows the chemical composition of iron powders, ratio of oxygen in easy-to-oxidize elements, hardness of particle cross-section, sintered body strength and variable range of dimensional changes of Examples 38–52 and Comparative Examples 28–31.

Any of Examples 38–52 exhibit a practically applicable green density and sintered body strength. Further, they exhibit an excellent dimensional accuracy with a variable range of dimensional changes of 0.1% or less.

With Example 51, where a small amount of easy-to-oxidize elements is contained, and Example 52, where a ratio of oxidization of easy-to-oxidize elements is 20 wt % or less, although dimensional accuracy was lowered, practically useful green density and sintered body strength were obtained.

Because a total amount of Si, Al, Ti and V in Comparative Examples 28 to 31 exceeds the upper limit of a proper range, only a low sintered body strength was obtained.

dried at 100°–300° C. in hydrogen, nitrogen or vacuum. The raw powders were screened to 250 µm or less without being annealed or reduced.

Green density, sintered body strength and variable range of dimensional changes of sintered body were measured by the same methods as those of Example 37.

Table 8-1 shows chemical compositions of iron powders of Examples 53–68 and Comparative Examples 32–38, and Table 8-2 shows atomizing conditions, drying conditions, ratios of oxidation of the easy-to-oxidize elements, powder hardness, ratios of the particles having a coefficient of configuration of 2.5 or less in the particles having a particle size of 75–106 µm or less, ratio of the particles having a particle size of –325 mesh (45 µm or less), and green density without finishing reduction, sintered body density and variable range of dimensional changes of these examples and comparative examples.

All of Examples 53–68 exhibit practically applicable green density and sintered body strength. Further, Examples 53–66 exhibit excellent dimensional accuracy with a variable range of dimensional changes of 0.1% or less.

With Example 67, where a ratio of oxidization of easy-to-oxidize elements is 20 wt % or less, and Example 68, where a small amount of easy-to-oxidize elements is con-

TABLE 7

Chemical composition of iron powder

|                        | Atomizing atmosphere | Drying condition | O <sub>2</sub> concentration (%) | Si (%) | Al (%) | Ti (%) | V (%)  | O (%) | Ratio of oxidization of easy-to-oxidize elements (%) | Powder hardness (HV (100)) | Green density (g/cm <sup>3</sup> ) | Tensile strength (kg/mm <sup>2</sup> ) | Variable range (%) |
|------------------------|----------------------|------------------|----------------------------------|--------|--------|--------|--------|-------|------------------------------------------------------|----------------------------|------------------------------------|----------------------------------------|--------------------|
| Example 38             | 0.5                  | 150° C.          | H <sub>2</sub>                   | 0.01   | <0.001 | <0.001 | <0.001 | 0.30  | 35                                                   | 115                        | 6.91                               | 40                                     | 0.10               |
| Example 39             | 0.5                  | 150° C.          | H <sub>2</sub>                   | 0.05   | <0.001 | <0.001 | <0.001 | 0.32  | 29                                                   | 115                        | 6.93                               | 40                                     | 0.09               |
| Example 40             | 0.5                  | 150° C.          | H <sub>2</sub>                   | 0.10   | <0.001 | <0.001 | <0.001 | 0.32  | 31                                                   | 120                        | 6.91                               | 41                                     | 0.09               |
| Example 41             | 0.5                  | 200° C.          | H <sub>2</sub>                   | 0.002  | 0.004  | <0.001 | <0.001 | 0.26  | 39                                                   | 130                        | 6.28                               | 40                                     | 0.09               |
| Example 42             | 0.5                  | 250° C.          | H <sub>2</sub>                   | 0.008  | 0.004  | <0.001 | <0.001 | 0.30  | 35                                                   | 128                        | 6.89                               | 45                                     | 0.10               |
| Example 43             | 0.1                  | 150° C.          | N <sub>2</sub>                   | 0.002  | 0.010  | <0.001 | <0.001 | 0.30  | 40                                                   | 135                        | 6.85                               | 44                                     | 0.08               |
| Example 44             | 1                    | 150° C.          |                                  | 0.002  | 0.05   | <0.001 | <0.001 | 0.31  | 24                                                   | 139                        | 6.82                               | 40                                     | 0.06               |
|                        |                      |                  | vacuum                           |        |        |        |        |       |                                                      |                            |                                    |                                        |                    |
| Example 45             | 2                    | 150° C.          | H <sub>2</sub>                   | 0.002  | <0.001 | 0.005  | <0.001 | 0.35  | 26                                                   | 135                        | 6.9                                | 42                                     | 0.05               |
| Example 46             | 1                    | 150° C.          | H <sub>2</sub>                   | 0.002  | <0.001 | 0.10   | <0.001 | 0.33  | 32                                                   | 130                        | 6.91                               | 41                                     | 0.07               |
| Example 47             | 0.2                  | 150° C.          | N <sub>2</sub>                   | 0.002  | <0.001 | <0.001 | 0.01   | 0.35  | 34                                                   | 135                        | 6.89                               | 42                                     | 0.08               |
| Example 48             | 0.3                  | 150° C.          | N <sub>2</sub>                   | 0.002  | <0.001 | <0.001 | 0.40   | 0.32  | 28                                                   | 135                        | 6.9                                | 41                                     | 0.07               |
| Example 49             | 0.5                  | 180° C.          | H <sub>2</sub>                   | 0.010  | <0.001 | <0.001 | 0.10   | 0.32  | 35                                                   | 130                        | 6.89                               | 40                                     | 0.09               |
| Example 50             | 0.5                  | 180° C.          | H <sub>2</sub>                   | 0.002  | 0.003  | 0.003  | 0.05   | 0.32  | 31                                                   | 120                        | 6.91                               | 41                                     | 0.10               |
| Example 51             | 0.5                  | 180° C.          | H <sub>2</sub>                   | 0.002  | <0.001 | <0.001 | <0.001 | 0.80  | 50                                                   | 150                        | 6.78                               | 40                                     | 0.21               |
| Example 52             | 6                    | 180° C.          | H <sub>2</sub>                   | 0.005  | 0.005  | <0.001 | 0.01   | 0.85  | 15                                                   | 220                        | 6.75                               | 41                                     | 0.20               |
| Comparative Example 28 | 0.3                  | 150° C.          | N <sub>2</sub>                   | 0.20   | 0.001  | 0.001  | 0.001  | 0.56  | 22                                                   | 210                        | 6.77                               | 32                                     | 0.12               |
| Comparative Example 29 | 0.03                 | 150° C.          | N <sub>2</sub>                   | 0.005  | 0.10   | 0.001  | 0.001  | 0.58  | 20                                                   | 180                        | 6.74                               | 33                                     | 0.11               |
| Comparative Example 30 | 0.3                  | 150° C.          | N <sub>2</sub>                   | 0.005  | 0.003  | 0.20   | 0.01   | 0.52  | 22                                                   | 190                        | 6.76                               | 31                                     | 0.10               |
| Comparative Example 31 | 0.3                  | 150° C.          | N <sub>2</sub>                   | 0.005  | 0.003  | 0.40   | 0.60   | 0.55  | 22                                                   | 190                        | 6.72                               | 31                                     | 0.12               |

## Examples 53–68, Comparative Examples 32–38

After having been refined in a converter or an electric furnace, molten metal containing C: 0.02 wt % or less, a content of each of Mn, Ni, Cr: 0.3 wt % or less, P: 0.002–0.02 wt %, S: 0.002–0.02 wt %, Mo: 6.0 wt % or less, Nb: 0.3 wt % or less, a total content of Si, V, Al, Ti and Zr: 1.5 wt % or less was prepared by use of a vacuum degassing apparatus. This molten metal was atomized with water having a pressure of 80–160 kgf/cm<sup>2</sup> in an atmosphere with an oxygen (O<sub>2</sub>) concentration of 10 vol % or less and then

tained, although dimensional accuracy was lowered, practically useful green density and sintered body strength were obtained.

Because a total amount of Si, Al, Ti and V in Comparative Examples 28 to 31 exceeds the upper limit of a proper range, only a low sintered body strength was obtained.

On the other hand, Comparative Examples 32–38 have a low green density or low sintered body strength because proper ranges of the present invention were exceeded.

The iron powder for powder metallurgy according to the present invention does not need an annealing step or a reducing process after the iron powder has been atomized with water, as has been needed for conventional water-atomized iron powder, so that the iron powder can be compacted in dies as a raw powder. Further, when the iron powder according to the present invention is sintered with the addition of Cu, graphite, the dimensional changes thereof caused in the sintering are less varied with respect to

the dispersion of added graphite as compared with conventional iron powder for powder metallurgy. As a result, a sintered body having excellent dimensional accuracy can be made, even allowing a sizing process to be omitted. Consequently, manufacturing of sintered parts can be simplified and shortened when the iron powder according to the present invention is used. Further, manufacturing cost of sintered parts can be decreased without damaging the characteristics of the product.

TABLE 8-1

|                    | Chemical composition of raw powder (wt %) |      |       |       |       |       |      |       |       |        |        |        |        |      |
|--------------------|-------------------------------------------|------|-------|-------|-------|-------|------|-------|-------|--------|--------|--------|--------|------|
|                    | C                                         | Mn   | Ni    | Cr    | P     | S     | Mo   | Nb    | Si    | V      | Al     | Ti     | Zr     | O    |
| Example 53         | 0.003                                     | 0.01 | 0.005 | 0.01  | 0.003 | 0.006 | 0.01 | 0.005 | 0.005 | <0.001 | 0.004  | <0.001 | <0.001 | 0.3  |
| Example 54         | 0.004                                     | 0.04 | 0.01  | 0.01  | 0.01  | 0.005 | 0.5  | 0.007 | 0.005 | <0.001 | 0.006  | <0.001 | <0.001 | 0.35 |
| Example 55         | 0.005                                     | 0.03 | 0.01  | 0.011 | 0.008 | 0.006 | 1.0  | 0.006 | 0.004 | <0.001 | 0.02   | <0.001 | <0.001 | 0.45 |
| Example 56         | 0.001                                     | 0.2  | 0.008 | 0.012 | 0.008 | 0.006 | 2.0  | 0.006 | 0.006 | <0.001 | 0.05   | <0.001 | <0.001 | 0.44 |
| Example 57         | 0.002                                     | 0.1  | 0.007 | 0.004 | 0.009 | 0.008 | 4.0  | 0.01  | 0.008 | <0.001 | 0.001  | <0.001 | <0.001 | 0.5  |
| Example 58         | 0.002                                     | 0.04 | 0.3   | 0.006 | 0.004 | 0.006 | 0.5  | 0.05  | 0.05  | 0.01   | 0.006  | <0.001 | <0.001 | 0.42 |
| Example 59         | <0.001                                    | 0.04 | 0.008 | 0.008 | 0.008 | 0.003 | 0.5  | 0.05  | 0.1   | <0.001 | 0.002  | <0.001 | <0.001 | 0.42 |
| Example 60         | 0.002                                     | 0.04 | 0.011 | 0.006 | 0.02  | 0.006 | 0.2  | 0.15  | 0.006 | 0.05   | 0.006  | <0.001 | <0.001 | 0.42 |
| Example 61         | 0.006                                     | 0.01 | 0.01  | 0.005 | 0.01  | 0.015 | 0.3  | 0.2   | 0.008 | 0.15   | <0.001 | <0.001 | <0.001 | 0.33 |
| Example 62         | 0.009                                     | 0.02 | 0.005 | 0.006 | 0.007 | 0.002 | 0.2  | 0.02  | 0.008 | 0.45   | <0.001 | <0.001 | <0.001 | 0.33 |
| Example 63         | 0.003                                     | 0.3  | 0.006 | 0.005 | 0.008 | 0.006 | 0.1  | 0.03  | 0.005 | 0.01   | 0.003  | 0.01   | <0.001 | 0.3  |
| Example 64         | 0.002                                     | 0.03 | 0.3   | 0.005 | 0.007 | 0.006 | 0.2  | 0.008 | 0.005 | 0.01   | 0.008  | 0.1    | <0.001 | 0.28 |
| Example 65         | 0.002                                     | 0.03 | 0.012 | 0.3   | 0.007 | 0.006 | 0.5  | 0.009 | 0.009 | 0.01   | 0.004  | <0.001 | 0.01   | 0.44 |
| Example 66         | 0.001                                     | 0.1  | 0.01  | 0.01  | 0.006 | 0.007 | 1.0  | 0.01  | 0.007 | 0.007  | 0.003  | <0.001 | 0.1    | 0.45 |
| Example 67         | 0.002                                     | 0.05 | 0.01  | 0.01  | 0.007 | 0.007 | 0.2  | 0.05  | 0.007 | 0.007  | 0.005  | 0.01   | 0.01   | 0.53 |
| Example 68         | 0.003                                     | 0.04 | 0.011 | 0.006 | 0.008 | 0.006 | 0.5  | 0.01  | 0.002 | <0.001 | <0.001 | <0.001 | <0.001 | 0.84 |
| Comparative ex. 32 | 0.022                                     | 0.09 | 0.008 | 0.01  | 0.01  | 0.009 | 0.2  | 0.007 | 0.002 | 0.007  | 0.01   | <0.001 | <0.001 | 0.42 |
| Comparative ex. 33 | 0.003                                     | 0.1  | 0.01  | 0.011 | 0.007 | 0.008 | 1.0  | 0.01  | 0.2   | 0.009  | 0.002  | <0.001 | <0.001 | 1.1  |
| Comparative ex. 34 | 0.003                                     | 0.1  | 0.01  | 0.01  | 0.011 | 0.007 | 0.4  | 0.3   | 0.01  | 0.6    | 0.007  | <0.001 | <0.001 | 0.59 |
| Comparative ex. 35 | 0.004                                     | 0.1  | 0.01  | 0.01  | 0.01  | 0.007 | 2.0  | 0.01  | 0.01  | 0.009  | 0.07   | <0.001 | <0.001 | 0.58 |
| Comparative ex. 36 | 0.005                                     | 0.02 | 0.005 | 0.005 | 0.007 | 0.002 | 0.2  | 0.02  | 0.02  | 0.015  | 0.008  | 0.2    | 0.005  | 0.5  |
| Comparative ex. 37 | 0.005                                     | 0.02 | 0.005 | 0.005 | 0.007 | 0.002 | 0.2  | 0.02  | 0.02  | 0.015  | 0.008  | 0.002  | 0.2    | 0.5  |
| Comparative ex. 38 | 0.002                                     | 0.11 | 0.011 | 0.009 | 0.011 | 0.008 | 0.1  | 0.008 | 0.008 | 0.01   | 0.01   | <0.001 | <0.001 | 1.5  |

TABLE 8-2

|                    | Atomizing conditions                      |                              |                                   | Ratio of                                  |                            |  | Number % of Particles having coefficient of configuration of 2.5 or less (Particle size 75-106 µm) | Particles through 3 25 mesh (-45 µm) | wt % of |
|--------------------|-------------------------------------------|------------------------------|-----------------------------------|-------------------------------------------|----------------------------|--|----------------------------------------------------------------------------------------------------|--------------------------------------|---------|
|                    | Atomizing atmosphere O2 concentration (%) | Atomizing pressure (kgf/cm2) | Drying conditions Gas Temperature | oxidation of easy-to-oxidize elements (%) | Powder hardness (Hv (100)) |  |                                                                                                    |                                      |         |
| Example 53         | 0.5                                       | 100                          | H2-180° C.                        | 35                                        | 115                        |  | 35                                                                                                 |                                      | 30      |
| Example 54         | 0.5                                       | 100                          | H2-180° C.                        | 34                                        | 120                        |  | 40                                                                                                 |                                      | 28      |
| Example 55         | 0.5                                       | 100                          | H2-180° C.                        | 25                                        | 125                        |  | 35                                                                                                 |                                      | 33      |
| Example 56         | 0.5                                       | 100                          | H2-180° C.                        | 28                                        | 130                        |  | 35                                                                                                 |                                      | 32      |
| Example 57         | 0.5                                       | 100                          | H2-130° C.                        | 30                                        | 137                        |  | 38                                                                                                 |                                      | 33      |
| Example 58         | 1                                         | 120                          | H2-180° C.                        | 45                                        | 138                        |  | 30                                                                                                 |                                      | 35      |
| Example 59         | 1                                         | 120                          | N2-150° C.                        | 49                                        | 140                        |  | 32                                                                                                 |                                      | 35      |
| Example 60         | 1                                         | 120                          | N2-150° C.                        | 35                                        | 135                        |  | 28                                                                                                 |                                      | 36      |
| Example 61         | 1                                         | 120                          | N2-150° C.                        | 50                                        | 150                        |  | 30                                                                                                 |                                      | 34      |
| Example 62         | 2                                         | 80                           | Vac.-150° C.                      | 33                                        | 175                        |  | 45                                                                                                 |                                      | 22      |
| Example 63         | 2                                         | 80                           | H2-280° C.                        | 38                                        | 135                        |  | 42                                                                                                 |                                      | 23      |
| Example 64         | 0.2                                       | 160                          | H2-280° C.                        | 25                                        | 130                        |  | 25                                                                                                 |                                      | 40      |
| Example 65         | 0.2                                       | 160                          | H2-280° C.                        | 35                                        | 120                        |  | 26                                                                                                 |                                      | 43      |
| Example 66         | 0.2                                       | 130                          | N2-150° C.                        | 36                                        | 110                        |  | 28                                                                                                 |                                      | 40      |
| Example 67         | 5                                         | 130                          | N2-150° C.                        | 15                                        | 125                        |  | 28                                                                                                 |                                      | 38      |
| Example 68         | 0.5                                       | 120                          | H2-180° C.                        | —                                         | 130                        |  | 25                                                                                                 |                                      | 35      |
| Comparative ex. 32 | 0.5                                       | 80                           | H2-180° C.                        | 38                                        | 280                        |  | 45                                                                                                 |                                      | 22      |
| Comparative ex. 33 | 0.5                                       | 80                           | N2-180° C.                        | 42                                        | 260                        |  | 42                                                                                                 |                                      | 22      |
| Comparative ex. 34 | 0.5                                       | 100                          | N2-180° C.                        | 38                                        | 270                        |  | 35                                                                                                 |                                      | 20      |
| Comparative ex. 35 | 0.5                                       | 100                          | N2-180° C.                        | 40                                        | 280                        |  | 36                                                                                                 |                                      | 21      |
| Comparative ex. 36 | 0.5                                       | 100                          | N2-180° C.                        | 36                                        | 270                        |  | 38                                                                                                 |                                      | 23      |

TABLE 8-2-continued

|                       | Atomizing conditions                                           |                                                 | Drying conditions<br>Gas Temperature | Ratio of<br>oxidation of<br>easy-to-oxidize<br>elements<br>(%) | Powder<br>hardness<br>(Hv (100)) | Number % of Particles<br>having coefficient of<br>configuration of 2.5 or less<br>(Particle size 75-106 $\mu$ m) | wt % of<br>Particles<br>through 3<br>25 mesh<br>(-45 $\mu$ m) |
|-----------------------|----------------------------------------------------------------|-------------------------------------------------|--------------------------------------|----------------------------------------------------------------|----------------------------------|------------------------------------------------------------------------------------------------------------------|---------------------------------------------------------------|
|                       | Atomizing<br>atmosphere<br>O <sub>2</sub> concentration<br>(%) | Atomizing<br>pressure<br>(kgf/cm <sup>2</sup> ) |                                      |                                                                |                                  |                                                                                                                  |                                                               |
| Comparative<br>ex. 37 | 0.5                                                            | 100                                             | N <sub>2</sub> -180° C.              | 35                                                             | 260                              | 35                                                                                                               | 30                                                            |
| Comparative<br>ex. 38 | 8                                                              | 100                                             | N <sub>2</sub> -180° C.              | 18                                                             | 190                              | 35                                                                                                               | 28                                                            |

TABLE 8-3

| Green density<br>compacted at<br>5t/cm <sup>2</sup><br>(Mg/m <sup>3</sup> ) | Sintered body strength<br>Sintered body density<br>6.8 Mg/m <sup>3</sup><br>(MPa) | Variable range<br>of dimensional<br>changes<br>(%) |
|-----------------------------------------------------------------------------|-----------------------------------------------------------------------------------|----------------------------------------------------|
| 53                                                                          | 6.85                                                                              | 420                                                |
| 54                                                                          | 6.87                                                                              | 560                                                |
| 55                                                                          | 6.89                                                                              | 615                                                |
| 56                                                                          | 6.91                                                                              | 735                                                |
| 57                                                                          | 6.83                                                                              | 820                                                |
| 58                                                                          | 6.82                                                                              | 550                                                |
| 59                                                                          | 6.8                                                                               | 545                                                |
| 60                                                                          | 6.9                                                                               | 595                                                |
| 61                                                                          | 6.82                                                                              | 605                                                |
| 62                                                                          | 6.79                                                                              | 500                                                |
| 63                                                                          | 6.86                                                                              | 510                                                |
| 64                                                                          | 6.87                                                                              | 515                                                |
| 65                                                                          | 6.88                                                                              | 555                                                |
| 66                                                                          | 6.89                                                                              | 605                                                |
| 67                                                                          | 6.88                                                                              | 520                                                |
| 68                                                                          | 6.8                                                                               | 520                                                |
| 32                                                                          | 6.67                                                                              | 410                                                |
| 33                                                                          | 6.68                                                                              | 380                                                |
| 34                                                                          | 6.65                                                                              | 375                                                |
| 35                                                                          | 6.66                                                                              | 350                                                |
| 36                                                                          | 6.68                                                                              | 395                                                |
| 37                                                                          | 6.68                                                                              | 355                                                |
| 38                                                                          | 6.69                                                                              | 390                                                |

What is claimed is:

1. Iron powder for powder metallurgy consisting essentially of a water atomized, non-heat treated iron powder containing C: 0.01 wt % or less, Mn: 0.30 wt % or less, Ni: 0.30 wt % or less, Cr: 0.30 wt % or less, Mo: about 5.0 wt % or less, Nb: about 0.20 wt % or less, a total of P and S: 0.05 wt % or less as impurities, at least one additional element that is more easily oxidizable than iron and wherein the balance is substantially Fe, wherein those of said particles having a particle size from about 75  $\mu$ m to about 106  $\mu$ m, include a portion having a coefficient of particle cross-sectional configuration of about 2.5 or less and are present in a numerical amount of about 10% or more,

said powder including particles having a particle size of about 45  $\mu$ m or less present in an amount of about 20 wt % or more, and having a particle cross section hardness of from about Hv 80 or higher to about 250 or lower,

said powder further having a particle surface covered with at least one oxide which is reducible in a sintering atmosphere,

15 and said surface having an oxygen content of about 1.0 wt % or less.

2. Iron powder further according to claim 1 wherein said additional element is present in a particle surface covered with oxide that is not reducible in the usual subsequent 20 sintering atmosphere.

25 3. Iron powder according to claim 2, wherein said element more easily oxidizable than iron includes one or two or more elements selected from the group consisting of Si: 0.01-0.1 wt %, Al: 0.003-0.05 wt %, V: 0.008-0.5 wt %, Ti: 0.003-0.1 wt % and Zr: 0.008-0.1 wt %.

4. Iron powder according to claim 3, wherein said additional elements are present in a total amount of about 0.003 to 0.5 wt %.

30 5. Iron powder for powder metallurgy consisting essentially of a water-atomized, non-heat treated iron powder containing C: 0.01 wt % or less, Mn: 0.30 wt % or less, Ni: 0.30 wt % or less, Cr: 0.30 wt % or less, Mo: about 5.0 wt % or less, Nb: about 0.20 wt % or less, a total of P and S: 0.05 wt % or less as impurities, at least one additional element present in a particle surface covered with oxide which is not reducible in a sintering atmosphere, said additional element selected from the group consisting of Al: 0.003-0.05 wt %, V: 0.008-0.5 wt %, Ti: 0.003-0.1 wt % and Zr: 0.008-0.1 wt % that is more easily oxidizable than iron and wherein the balance is substantially Fe, wherein those of said particles having a particle size from about 75  $\mu$ m to about 106  $\mu$ m, include a portion having a coefficient of particle cross-sectional configuration of about 2.5 or less and the amount of said portion is about 10% or more in said particles,

45 40 said powder including particles having a particle size of about 45  $\mu$ m or less present in an amount of about 20 wt % or more, and having a particle cross section hardness of from about Hv 80 or higher to about 250 or lower,

45 said powder further having a particle surface covered with at least one oxide which is reducible in a sintering atmosphere,

50 and said surface having an oxygen content of about 1.0 wt % or less.

\* \* \* \* \*

UNITED STATES PATENT AND TRADEMARK OFFICE  
**CERTIFICATE OF CORRECTION**

PATENT NO. : 5,534,045

DATED : July 9, 1996

INVENTOR(S) : Kuniaki Ogura, Hiroyuki Ishikawa, Yoshiaki Maeda and  
Kouichi Komamura

It is certified that error appears in the above-identified patent and that said Letters Patent is hereby  
corrected as shown below:

In Column 1, line 51, please change "atomizod" to  
--atomized--.

In Column 8, line 8, please change "atomizod" to  
--atomized--.

In Column 13, line 27, please change "N<sub>s</sub>" to --N<sub>2</sub>--.

Signed and Sealed this  
Tenth Day of December, 1996

Attest:



BRUCE LEHMAN

Attesting Officer

Commissioner of Patents and Trademarks